

R. HAZELTINE.

PROCESS OF COATING IRON AND STEEL SHEETS WITH LEAD AND LEAD ALLOYS.

APPLICATION FILED FEB. 9, 1914.

1,161,475.

Patented Nov. 23, 1915.



WITNESSES

*W. S. Rodgers*  
*H. F. Steffens*

INVENTOR

R. HAZELTINE

BY *H. E. Daniels*  
ATTORNEY

# UNITED STATES PATENT OFFICE.

REGINALD HAZELTINE, OF WHEELING, WEST VIRGINIA, ASSIGNOR TO WHEELING CORRUGATING COMPANY, OF WHEELING, WEST VIRGINIA, A CORPORATION OF WEST VIRGINIA.

## PROCESS OF COATING IRON AND STEEL SHEETS WITH LEAD AND LEAD ALLOYS.

1,161,475.

Specification of Letters Patent. Patented Nov. 23, 1915.

Application filed February 9, 1914. Serial No. 817,467.

To all whom it may concern:

Be it known that I, REGINALD HAZELTINE, a citizen of the United States of America, and resident of Wheeling, county of Ohio, 5 and State of West Virginia, have invented certain new and useful Improvements in Processes of Coating Iron and Steel Sheets with Lead and Lead Alloys, of which the following is a specification.

This invention relates to the art or process 10 of coating iron and steel sheets or plates with lead or with alloy mixtures wherein high percentages of lead are employed.

As is well known, the coating of iron and 15 steel sheets or plates with metal is commonly accomplished by directing the same through a pot in which they are first passed through a suitable flux, thence through the coating metal which is in a liquid state, and thence 20 outward through rolls working in palm oil. It has hitherto been impracticable, however, to employ said process in the coating of sheets with lead or with alloys containing high percentages of lead, due to the fact that 25 the surfaces of the iron or steel rolls invariably employed in the pots for effecting the coating do not become coated with such coating metal, lead not having an affinity for iron or steel in the presence of palm oil; and, 30 consequently, a satisfactory lead or lead-alloy coating cannot thereby be applied to the sheets.

My invention contemplates the employment of rolls, the outer surfaces of which 35 are composed of a non-ferrous metal, as brass, bronze, nickel, copper, or monel metal, which, instead of repelling a tendency to become coated in the presence of palm oil, as do iron and steel rolls, readily take or acquire a coating of lead or of a high percentage 40 lead alloy, said rolls being submerged or partially submerged in the palm oil of a pot containing the lead or alloy in liquid form. The sheets to be coated are passed through, 45 or between, said non-ferrous rolls after having passed through the fluid coating metal in the pot, and, in so passing through, said rolls act to smooth the coating on, and impart an even finish to, the surfaces of the 50 sheets, causing the latter to emerge free from dirt and scruff.

Referring to the accompanying drawing, in which the figure is a longitudinal section of a preferred form of apparatus by means

of which my process may be carried out, 1 55 indicates a coating pot of a common type containing the molten metal 2 with which the sheets are to be coated. Overlying said metal at the delivery end of the pot is a quantity of palm oil or other suitable grease 60 or flux 3. Mounted in said delivery end of the pot so as to be submerged, or partially submerged, in said flux 3 and to also contact with the coating metal 2 is a set of rolls 4 having non-ferrous surfaces. Said rolls 65 may be composed wholly of non-ferrous metal, or they may have only their outer, or sheet-engaging, surfaces composed of such metal.

While tin is ordinarily used in connection 70 with lead for producing a suitable metal coating alloy, such, if and when used in the present process, is employed only in extremely small proportions, or in a proportion amounting to less than five per centum 75 of the whole, in view of the fact that tin, in other than relatively small proportions, has a decided tendency to quickly dissolve or deteriorate brass or bronze or alloys of said metals. 80

I would have it understood that the term "non-ferrous," as herein used, does not necessarily exclude rolls composed of alloy metals in the composition of which iron enters in non-deleterious proportions, as it 85 is possible that rolls which will take a lead coating in the presence of palm oil may be made of an alloy containing some iron. By "non-ferrous," I therefore mean a metal which possesses the coating characteristics 90 of such non-ferrous metals as brass, bronze and nickel, and not those of iron and steel.

What I claim is—

1. The art of coating iron and steel sheets with alloys wherein lead is the chief constituent, which consists in passing said sheets from the coating bath to and through a suitable overlying flux, and in directing said sheets, during their passage through said flux, between coating-contacting rolls 100 submerged in said flux and composed of a metal which has an affinity for said alloy in the presence of said flux. 95

2. The art of coating iron and steel sheets with lead alloys, which consists in passing 105 said sheets through the coating bath and an overlying bath of palm oil, and in subjecting said sheets, during their passage through the

palm oil, to the action of a coating-acquiring set of rolls submerged in said oil and having surfaces composed of a non-ferrous metal which has an affinity for said alloy in the presence of palm oil.

3. The art or process of coating iron and steel sheets, which consists in passing said sheets, first, through a high percentage lead alloy in liquid form, and thence through a suitable flux which overlies said alloy, and in subjecting said sheets, during their passage through said flux, to the action of a set of rolls having non-ferrous surfaces submerged in said flux and disposed in contact with said alloy.

4. The art of coating iron and steel sheets with high percentage lead mixtures, which consists in passing said sheets from the coating bath to and between a set of rolls having surfaces composed of a non-ferrous metal,

said rolls being submerged in a flux which overlies said coating bath and having their under surfaces in contact with said bath.

5. The art of coating iron and steel sheets with lead alloys, which consists in passing said sheets from the coating bath of said alloy in liquid form to and through a set of rolls whose surfaces are composed of an alloy for which lead has an affinity in the presence of palm oil, said rolls being disposed with their under surfaces in contact with said alloy and with their meeting point submerged in palm oil overlying said alloy.

In testimony whereof, I affix my signature in presence of two subscribing witnesses.

REGINALD HAZELTINE.

Witnesses:

J. B. SCOTT,  
L. B. VOGLER.